

J. H. BUTLER,  
PROCESS OF MAKING COATED LEATHER ARTICLES,  
APPLICATION FILED OCT. 22, 1914.

1,236,049.

Patented Aug. 7, 1917.



Fig. 1. 1 2



Fig. 2.

Fig. 4.

Fig. 5.



Fig. 3.

Witnesses  
H. Lowenstein  
James H. Marr.

Inventor  
James H. Butler  
By  
Edward E. Cleland  
Attorney

# UNITED STATES PATENT OFFICE.

JAMES H. BUTLER, OF GLOVERSVILLE, NEW YORK. ASSIGNOR OF ONE-HALF TO FRANK W. AUSTIN, OF GLOVERSVILLE, NEW YORK.

## PROCESS OF MAKING COATED LEATHER ARTICLES.

1,236,049.

Specification of Letters Patent. Patented Aug. 7, 1917.

Application filed October 22, 1914. Serial No. 868,096.

*To all whom it may concern:*

Be it known that I, JAMES H. BUTLER, a citizen of the United States, residing at Gloversville, in the county of Fulton and State of New York, have invented certain new and useful Improvements in Processes of Making Coated Leather Articles, of which the following is a specification, reference being had therein to the accompanying drawing.

My invention relates to the manufacture of leather and leather articles, and has for its object the production of an improved process for coating leather in order to impart to it water-proof and insulating properties.

The principal novel feature of this invention consists in the vulcanization of rubber directly to leather, and the coating thereby of the leather without destroying its elasticity. The leather is treated after the usual process of preparing the hide, by extracting the oil and dressing the leather in such manner that it will retain its pliability. The oil is removed as a preliminary to filling the pores with rubber and vulcanizing the same therein.

In carrying out my process, so-called washable leather is coated with liquid rubber, that is to say, a rubber solution which penetrates the pores and covers the surface, and this is vulcanized upon the leather as a unit by means of appliances to be presently referred to. The washable leather or so-called "washable" process of tanning upon which my invention is based, depends upon a secret combination of chrome with fat liquid. Consequently, the skins which I use are tanned with a grease. This procedure of combining chrome with oil, which produces a washable leather, while not in itself of my invention, I believe to be purely an American process not heretofore known or used abroad.

I am aware that it was proposed, in the provisional British patent specification, No. 18673, dated August 25, 1902, to coat leather with india rubber by deposition out of a solution; but this applies to a different kind of leather. Such degreased chrome leather is not soft and pliable, could not be substituted for oil treated leather, and will not stand the process of vulcanizing without destroying the pliability of the leather which, in my invention, is preserved.

The practice of my invention, and a glove

produced thereby, are illustrated in the accompanying drawings, in which—

Figure 1 shows a section of a piece of leather coated according to my process. 60

Fig. 2 shows one form of glove produced by my process turned inside out.

Fig. 3 is a longitudinal sectional view of a glove with vulcanizing dies in place.

Figs. 4 and 5 are detailed sectional views 65 of seams illustrating different methods of making the same.

In practising my process, I take a tanned leather 1 (Fig. 1) produced by the so-called "washable" process which, as stated, consists 70 of treatment with a combination of chrome with fat-liquor or oil, remove traces of oil, if desired, with gasolene or similar solvent, then coat the flesh side 2 of the leather with a solution of raw rubber 3 which may be 75 made in gasolene or other well known volatile solvent available for this purpose. This coating is allowed to dry by evaporation, leaving a deposit upon the leather and in the pores of the same, as indicated in Fig. 1. 80 I then apply raw sheet rubber 4 to the prepared surface of the leather and the rubber coating deposited thereon. For this purpose I may and do use 5-minute-cure rubber, and vulcanize in an oven heated with 85 sixty pounds of steam. The raw rubber sheet 4 softens, flows, and unites with the rubber solution 3 previously deposited on the leather, so that all the pores of the leather contain filaments of the rubber, and 90 the surfaces of the two materials are strongly adherent. The result, after vulcanizing, is a unified and integral sheet or material which may be handled and worked the same as enameled or other coated 95 leather.

Figs. 2 to 5, inclusive, illustrate the use of this invention as applied to a glove. It will be noticed that the leather has previously been treated as described for the general 100 process, to remove traces of oil. I might add that any other preliminary steps may be followed in the preparation of the leather which the condition of the material or general experience may show to be necessary or 105 expedient.

The leather 1 thus prepared is cut according to the proper patterns for the glove to be made. The sheet rubber 4 is cut in the same manner as the leather and after the coated 110 leather is dry, these rubber pattern pieces are laid upon the corresponding leather

pieces, so as to register therewith, the parts are stitched together, all the seams are reinforced with overlapping rubber strips 5 secured in place by rubber cement (consisting preferably of a simple solution of raw rubber in a volatile solvent), the glove is turned right side out as shown in Fig. 3, French chalk put in the glove to cover the surface of the rubber and prevent the same from sticking to the mold when heated, and the heated molds are then inserted, as also shown in Fig. 3, and the glove is placed in an oven. Here it is exposed to heat produced by steam or hot air and kept at vulcanizing temperature until the rubber is entirely cured and all the constituents are reduced to a homogeneous, continuous and integral tissue. This part of the process I have carried on very successfully with a vulcanizing heat of 60 pounds of steam, used for twenty minutes. As stated in the description of the general process, however, this time may vary, as rubber containing sulfur may be prepared in sheets so that it will cure in five minutes, in an oven heated with sixty pounds of steam. The exact time of exposure is, therefore, to be determined by the operator according to the material employed and the results desired. The slower cure may produce a tougher lining, while the quicker cure may have its effect on the final appearance of the leather.

The structural details of the glove or other article to be produced are, of course, not claimed, and need not be specifically de-

scribed herein. Suitable seams are shown in Figs. 4 and 5, the first with, and the second without, a covering strip 5 of raw rubber ready to be vulcanized into a coherent and integral tissue.

Having thus described my invention, what I claim, and desire to secure by Letters Patent is:

The process of producing a pliable, waterproof, and insulating hollow leather article which consists in first treating the leather to remove the oil and open its pores, on the surface to be inside the article, turning the leather tissue inside out, coating the then outer surface of the leather and filling the pores thereof with a solution of raw rubber, evaporating the solvent therefrom, applying overlapping sheets of raw or uncured rubber thereto, so as to completely cover the leather surface, turning the article again, so as to bring the rubber coating inside, inserting suitable heating dies, and exposing the entire article to a vulcanizing temperature, both from within and without, whereby will be produced a leather integument interiorly coated with a homogeneous and continuous rubber surface practically integral with the leather fabric.

In testimony whereof I affix my signature in presence of two witnesses.

JAMES H. BUTLER.

Witnesses:

JOHN TREHER,  
ANNIE I. AUSTIN.